# EUROPEAN PATENT APPLICATION

(11) **EP 4 782 565 A1**
(43) Date of publication of application: **29.07.2026**
(21) Application number: 24926992.9
(22) Date of filing: 09.12.2024
(51) Int. Cl.: C23C 2/06, C22C 18/00, C23C 2/26, C23C 2/40

(54) **ZN-AL-MG-BASED PLATED STEEL SHEET**

(30) Priority: 27.02.2024 JP 2024027843
(71) Applicant: JFE Steel Corporation, Tokyo 100-0011 (JP)
(72) Inventor: OGAWA, Shuhei, Tokyo 100-0011 (JP); FUKATA, Tsuyoshi, Tokyo 100-0011 (JP)
(74) Representative: Scott, Stephen John
(86) International application number: PCT/JP2024/043478
(87) International publication number: WO 2025/182227

(57) **Abstract**

Provided is a Zn-Al-Mg coated steel sheet having excellent post-painting corrosion resistance and painting layer adhesion. The Zn-Al-Mg coated steel sheet includes a base steel sheet and a coated layer formed on at least one side of the base steel sheet. The coated layer has a chemical composition, in mass%, containing Al: 0.5 % to 3.5 % and Mg: 0.5 % to 3.5 %, with the balance being Zn and inevitable impurities. The surface of the coated layer has a microstructure including a single-phase Zn microstructure and a eutectic microstructure. The eutectic microstructure includes a Zn-Mg intermetallic compound phase and a Zn phase, and optionally includes either or both of an Al phase and an Al-Mg intermetallic compound phase. The coating weight of the coated layer is 35 g/m² to 80 g/m². An average oxide film thickness at the surface of the coated layer is 50 nm or less. When an average value of oxygen intensity at the surface of the coated layer is taken as 1, a standard deviation σ of the oxygen intensity is 0.30 or less.

## Description

### TECHNICAL FIELD

The present disclosure relates to Zn-Al-Mg coated steel sheets.

### BACKGROUND

Conventionally, hot-dip galvanized steel sheets have excellent sacrificial protection and good corrosion resistance, and therefore have been utilized as anti-corrosion steel sheets for automobiles. However, with the globalization of the automotive market, the need for coated steel sheets having higher corrosion resistance is increasing due to factors such as improved quality requirements in emerging countries and worsening corrosion environments caused by air pollution. Under these circumstances, the adoption of Zn-Al-Mg coated steel sheets, which have improved corrosion resistance due to the addition of elements such as aluminum (Al) and magnesium (Mg) to a zinc coating, is expanding. Further, various technologies have been developed to further improve corrosion resistance and achieve both corrosion resistance and other properties by controlling factors such as the composition of the coating and the method of producing the coating.

In Patent Literature (PTL) 1, a coated steel material is described in which Al content in the coating is 0.5 % to 14 % and Mg content is 0.5 % to 5 %, thereby limiting the Mg content on the coated surface and improving wear resistance and anti-white rust property. In PTL 2, a zinc alloy coated steel material is described in which Al content in the coating is 0.1 % to 5.0 % and Mg content is 0.1 % to 5.0 %, and a defined structure is present between the steel substrate and the coated layer, thereby improving weldability and worked portion corrosion resistance.

Further, when Zn-Al-Mg coated steel sheets are used in automobiles, the sheets undergo chemical conversion treatment and electrodeposition coating. While phosphate-based chemical conversion treatments are commonly used, the adoption of Zr chemical conversion treatments has been increasing among OEMs in recent years, with the aim of sludge reduction and decreasing phosphorus levels in waste liquid.

### CITATION LIST

### Patent Literature

PTL 1: JP 2019-501296 A
PTL 2: JP 2018-506644 A
PTL 3: JP 2014-162957 A

### SUMMARY

### (Technical Problem)

Unlike conventional hot-dip galvanized steel sheets, Zn-Al-Mg coated steel sheets have various eutectic microstructures having different oxide film thicknesses depending on the coating composition, production conditions, and the like, resulting in a non-uniform microstructure on the coated surface. When Zr chemical conversion treatment is applied to such surfaces, the removal of the oxide film by etching becomes uneven across the microstructure, resulting in the formation of a non-uniform Zr chemical conversion layer on the coated surface. This leads to problems such as a decrease in corrosion resistance and painting layer adhesion after electrodeposition coating.

In PTL 3, a method is described of producing a coated steel material in which the uniformity of the Zr chemical conversion layer is improved by adjusting the composition of the Zr chemical conversion treatment bath. However, restricting the composition of the Zr chemical conversion treatment bath could lead to a decrease in robustness and potentially affect the conversion properties of materials other than Zn-Al-Mg coated steel sheets, raising production concerns. Therefore, there was a need for a Zn-Al-Mg coated steel sheet having a uniform oxide film that could form a uniform Zr chemical conversion layer regardless of the composition of the Zr chemical conversion treatment bath.

In view of the above issues, it would be helpful to provide a Zn-Al-Mg coated steel sheet that has a thin, uniform oxide film formed at the surface of the Zn-Al-Mg coated sheet and has excellent post-painting corrosion resistance and painting layer adhesion.

### (Solution to Problem)

In order to solve the aforementioned problems, the inventors conducted intensive studies and made the following discoveries. In a Zn-Al-Mg coated steel sheet, the coated layer has a microstructure that includes a single-phase Zn microstructure and a eutectic microstructure having a defined phase. Further, by setting coating weight, average oxide film thickness, and the standard deviation σ of oxygen intensity at the surface of the coated layer within defined ranges, the post-painting corrosion resistance and the painting layer adhesion can be improved. Further, when producing a Zn-Al-Mg coated steel sheet, by cooling in a defined temperature range after gas wiping with a defined atmosphere and cooling rate, the Zn-Al-Mg coated steel sheet described above can be obtained.

Primary features of the present disclosure are as follows.
[1] A Zn-Al-Mg coated steel sheet comprising a base steel sheet and a coated layer formed on at least one side of the base steel sheet,
   wherein the coated layer has a chemical composition, in mass%, containing (consisting of) Al: 0.5 % to 3.5 % and Mg: 0.5 % to 3.5 %, with the balance being Zn and inevitable impurities,
   wherein a surface of the coated layer has a microstructure comprising a single-phase Zn microstructure and a eutectic microstructure,
   wherein the eutectic microstructure comprises a Zn-Mg intermetallic compound phase and a Zn phase, and optionally comprises either or both of an Al phase and an Al-Mg intermetallic compound phase,
   wherein the coating weight of the coated layer is 35 g/m² to 80 g/m²,
   wherein an average oxide film thickness at the surface of the coated layer is 50 nm or less,
   and wherein, when an average value of oxygen intensity at the surface of the coated layer is taken as 1, a standard deviation σ of the oxygen intensity is 0.30 or less.
[2] The Zn-Al-Mg coated steel sheet according to [1], above, wherein the chemical composition of the coated layer further contains one or more selected from the group consisting of Si, Fe, Pb, Ti, Ni, Cu, Co, Mn, Cr, Mo, V, Sr, B, Bi, Cd, Sn, and REM, in a total amount of 1.0 mass% or less.

### (Advantageous Effect)

According to the present disclosure, it is possible to provide a Zn-Al-Mg coated steel sheet having excellent post-painting corrosion resistance and painting layer adhesion.

### BRIEF DESCRIPTION OF THE DRAWINGS

In the accompanying drawings:
FIG. 1 is an SEM image of a surface of a coated layer of an Example (No. 1) according to an embodiment of the present disclosure.

### DETAILED DESCRIPTION

The following is a description of an embodiment of the Zn-Al-Mg coated steel sheet according to the present disclosure. The embodiments described below are example embodiments of the present disclosure, and do not limit configuration to the specific examples described.

### [Zn-Al-Mg coated steel sheet]

The Zn-Al-Mg coated steel sheet according to an embodiment of the present disclosure includes a base steel sheet and a coated layer formed on at least one side of the base steel sheet. Further, the coated layer has a chemical composition, in mass%, consisting of Al: 0.5 % to 3.5 % and Mg: 0.5 % to 3.5 %, with the balance being Zn and inevitable impurities, and the surface of the coated layer has a microstructure including a single-phase Zn microstructure and a eutectic microstructure. Further, the eutectic microstructure contains a Zn-Mg intermetallic compound phase and a Zn phase, and optionally contains either or both of an Al phase and an Al-Mg intermetallic compound phase. The coated layer coating weight is 35 g/m² to 80 g/m², an average oxide film thickness at the surface of the coated layer is 50 nm or less, and, when an average value of oxygen intensity at the surface of the coated layer is taken as 1, the standard deviation σ of the oxygen intensity is 0.30 or less.

### [Base steel sheet]

There are no particular limitations on the type of base steel sheet. Typical hot-rolled steel sheets or cold-rolled steel sheets, such as ultra-low-carbon mild steel, can be used. There is no particular limitation on the thickness of the base steel sheet. The thickness of the base steel sheet is preferably 0.7 mm or more. The thickness of the base steel sheet is preferably 2.0 mm or less. The coated layer may be formed on one side of the base steel sheet, or on both sides.

### [Chemical composition of coated layer]

The following describes the chemical composition of the coated layer.

When the Al content in the coated layer is less than 0.5 mass%, post-painting corrosion resistance and painting layer adhesion cannot be secured. Further, a large amount of dross is generated in the coating bath due to the oxidation of Mg. The Al content in the coated layer is therefore 0.5 mass% or more. The Al content in the coated layer is preferably 1.0 mass% or more. On the other hand, when the Al content in the coated layer exceeds 3.5 mass%, an Al phase or an Al-rich Al-Zn phase precipitates as the primary crystal. The Al phase or Al-rich Al-Zn phase preferentially corrodes in the coated layer, but unlike the Zn-Mg intermetallic compound phase, does not stabilize corrosion products and improve corrosion resistance and instead decreases post-painting corrosion resistance. Therefore, when the Al content in the coated layer is 3.5 mass% or less, a coating microstructure having a Zn phase as the primary crystal and a eutectic microstructure described later are obtainable. The Al content in the coated layer is therefore 3.5 mass% or less. The Al content in the coated layer is preferably 3.0 mass% or less.

When the Mg content in the coated layer is less than 0.5 mass%, post-painting corrosion resistance cannot be secured. Further, when the Mg content in the coated layer is 1.0 mass% or more, the Zn-Mg intermetallic compound phase is stably dispersed in the eutectic microstructure of the coated layer, and post-painting corrosion resistance improves with increasing Mg content, which is preferable. The Mg content in the coated layer is therefore 0.5 mass% or more. The Mg content in the coated layer is preferably 1.0 mass% or more. On the other hand, when the Mg content in the coated layer exceeds 3.5 mass%, a Zn phase or a Zn-Mg intermetallic compound phase precipitates as the primary crystal. The Zn-Mg intermetallic compound phase is more easily oxidized than the Zn phase, and therefore the oxide film that forms tends to be thicker, decreasing the painting layer adhesion of electrodeposition coating to a Zr chemical conversion treatment substrate. The Mg content in the coated layer is therefore 3.5 mass% or less. The Mg content in the coated layer is preferably 2.0 mass% or less.

The coated layer may contain, as optional additives, one or more selected from the group consisting of Si, Fe, Pb, Ti, Ni, Cu, Co, Mn, Cr, Mo, V, Sr, B, Bi, Cd, Sn, and REM (rare earth metals), in a total amount of 1.0 mass% or less. When the total content of these elements exceeds 1.0 mass%, operational problems due to instability of the coating bath composition or quality problems that impair surface appearance become more likely. Therefore, when one or more selected from the group consisting of Si, Fe, Pb, Ti, Ni, Cu, Co, Mn, Cr, Mo, V, Sr, B, Bi, Cd, Sn, and REM are included, the total content of these elements is 1.0 mass% or less. A lower limit of the content is not particularly limited and may be 0.0 mass%.

The balance of the chemical composition of the coated layer consists of Zn and inevitable impurities.

### [Microstructure of coated layer]

The following describes the microstructure of the coated layer. The microstructure of the coated layer described below refers to the microstructure at the surface of the coated layer.

The coated layer according to the present disclosure has a microstructure that includes a single-phase Zn microstructure and a eutectic microstructure. The single-phase Zn microstructure is necessary for Zn to exert its sacrificial protection effect in the coated layer, and good post-painting corrosion resistance can be obtained when the coated layer has the single-phase Zn microstructure.

The eutectic microstructure contained in the coated layer includes a Zn-Mg intermetallic compound phase and a Zn phase, and optionally also includes either or both of an Al phase and an Al-Mg intermetallic compound phase. Here, Zn-Mg intermetallic compound phases are intermetallic compound phases consisting mainly of Zn and Mg, such as MgZn₂, MgZn₁₁, Mg₂Zn₃, and MgZn. Further, Al-Mg intermetallic compound phases are intermetallic compound phases consisting mainly of Al and Mg, such as Mg₂Al₃, MgAl, and Mg₁₇Al₁₂. Such eutectic microstructures preferentially corrode during a corrosion process of the coated layer. The Mg eluted from the eutectic microstructure during corrosion stabilizes the corrosion products, mainly oxides or hydroxides in the coated layer, and inhibits subsequent corrosion of the coated layer overall. That is, the presence of the eutectic microstructure in the coated layer allows for good post-painting corrosion resistance.

The presence or absence of a single-phase Zn microstructure and a eutectic microstructure on the coated surface can be confirmed by combining observation of reflected electron images using a scanning electron microscope (SEM) and compositional analysis using an energy-dispersive X-ray analyzer (EDX) attached to the SEM or analysis using an electron probe microanalyzer (EPMA), as follows. FIG. 1 illustrates an SEM image of the coated layer surface of an Example according to an embodiment of the present disclosure (No. 1, described later). In FIG. 1, the regions that have a smooth, white appearance are Zn phase, and in these regions, only Zn is detected by EDX or EPMA. These regions are therefore judged to be the single-phase Zn microstructure 10. In FIG. 1, the region having a lamellar microstructure is the eutectic microstructure 20. In this region, the white portions are Zn phase, and the gray areas are either Zn-Mg intermetallic compound phase, Al phase, or Al-Mg intermetallic compound phase. When Zn and Mg are detected in the eutectic microstructure 20 by EDX or EPMA, it is judged that the eutectic microstructure 20 contains a Zn-Mg intermetallic compound phase and a Zn phase. When Al is further detected in the eutectic microstructure 20 by EDX or EPMA, it is judged that the eutectic microstructure 20 contains either or both an Al phase and an Al-Mg intermetallic compound phase.

### [Coated layer coating weight: 35 g/m² to 80 g/m²]

The inventors discovered that in Zn-Al-Mg coating, the phase structure in the coating surface changes depending on the coating weight. Specifically, it was confirmed that the single-phase Zn microstructure tends to grow in an ellipsoidal shape with the minor axis length in the thickness direction of the base steel sheet and the major axis length in the horizontal direction of the base steel sheet. As the coating weight increases, eutectic microstructure is more likely to interpose between the single-phase Zn microstructure and the coating surface in the minor axis length of the slow-growing single-phase Zn microstructure, and the area proportion of the eutectic microstructure on the coating surface increases. The eutectic microstructure contains metals less noble than Zn, such as Mg and Al, and is therefore easily oxidized, and an increase in the area proportion of the eutectic microstructure on the coated surface increases the average oxide film thickness, as described later. When the coating weight of the coated layer exceeds 80 g/m², post-painting corrosion resistance improves, but the average oxide film thickness becomes too thick, inhibiting the formation of the Zr chemical conversion layer and resulting in poor painting layer adhesion. The coating weight of the coated layer is therefore 80 g/m² or less. On the other hand, when the coating weight of the coated layer is less than 35 g/m², the period during which the coated layer exhibits sacrificial protection is decreased, and therefore post-painting corrosion resistance cannot be secured. The coating weight of the coated layer is therefore 35 g/m² or more.

The coating weight of the coated layer can be determined in accordance with JIS H 0401:2021. Specifically, the coated layer can be dissolved and removed from the coated steel sheet using hydrochloric acid, and the difference in weight of the steel sheet before and after dissolution can be determined.

### [Average oxide film thickness at surface of coated layer is 50 nm or less]

When the average oxide film thickness at the surface of the coated layer exceeds 50 nm, the surface is not sufficiently etched during the Zr chemical conversion treatment, suppressing the formation of the Zr chemical conversion layer and decreasing the painting layer adhesion. Further, depending on the coating weight of the coated layer, post-painting corrosion resistance may not be secured. The average oxide film thickness at the surface of the coated layer is therefore 50 nm or less. On the other hand, when the average oxide film thickness is extremely thin, production and storage costs increase, and therefore the average oxide film thickness at the surface of the coated layer is preferably 2 nm or more.

The average oxide film thickness at the surface of the coated layer can be determined using an X-ray fluorescence spectrometer as follows. The tube voltage is set to 30 kV, the current to 100 mA, the collimator diameter to 30 mm, and the spectroscopic crystal to TAP. O-Kα radiation is then measured at the surface of the test material. For the detected O-Kα radiation, intensity at a background position is also measured in addition to a peak position, and the net intensity of O-Kα radiation is calculated. In addition to the test material, silicon wafers with silicon oxide films of different thicknesses are measured under the same conditions as reference samples, and a calibration curve is created between the oxide film thickness and the O-Kα radiation intensity. Reference samples with oxide film thicknesses of approximately 1/2, 1, and 2 times 50 nm (for example, 24 nm, 54 nm, and 96 nm) can be used. The integration time for each measurement is 20 s or longer. Using the created calibration curve, the measurement results on the test material are calculated as the oxide film thickness in terms of silicon oxide film, and the obtained result is taken as the average oxide film thickness.

### [When average value of oxygen intensity on surface of coated layer is taken as 1, standard deviation σ of oxygen intensity is 0.30 or less]

As a result of intensive studies by the inventors, it was discovered that, in addition to controlling the average oxide film thickness as described above, decreasing variation in oxide film thickness on the coated surface leads to improvements in post-painting corrosion resistance and painting layer adhesion. As described above, in Zn-Al-Mg coated steel sheets produced by conventional methods, the difference in oxide film thickness between the single-phase Zn microstructure and the eutectic microstructure (variation in oxide film thickness) becomes large. When a Zr chemical conversion treatment is applied to such coated steel sheets, etching of the oxide film takes longer on the eutectic microstructure than on the single-phase Zn microstructure, and the reaction time for the formation of the Zr chemical conversion layer is decreased. As a result, the Zr chemical conversion layer on the eutectic microstructure is thinner than that on the single-phase Zn microstructure. When electrodeposition coating is applied in this state and the post-painting corrosion resistance or the painting layer adhesion is evaluated, the eutectic microstructure where the Zr chemical conversion layer is thin acts as the weakest point, becoming the initiation point for corrosion or paint layer peeling, and therefore excellent results cannot be obtained. Therefore, the inventors defined the difference in oxide film thickness between the single-phase Zn microstructure and the eutectic microstructure as "the standard deviation σ of the oxygen intensity when the average value of the oxygen intensity at the surface of the coated layer is taken as 1", and investigated the conditions for improving corrosion resistance and post-painting adhesion. The inventors discovered that a significant effect occurs when σ is 0.30 or less. Therefore, when the average value of the oxygen intensity at the surface of the coated layer is taken as 1, the standard deviation σ of the oxygen intensity is 0.30 or less. A lower limit of the standard deviation σ is not particularly limited, and is generally 0.10 or higher.

The standard deviation σ of the oxygen intensity at the surface of the coated layer, with the average value of the oxygen intensity taken as 1, can be determined as follows. The measuring device used is EPMA-1720HT, produced by Shimadzu Corporation. During measurement, the accelerating voltage is 15 kV, the beam current is 80 nA, and the integration time is 40 ms/point. Oxygen intensity in a 180 µm × 180 µm field of view of the surface of the test material is measured by mapping, and dot data is acquired. The average value and standard deviation of all acquired dot data are calculated, and a value obtained by dividing the standard deviation by the average value is defined as the standard deviation σ.

### [Method of producing Zn-Al-Mg coated steel sheet]

The following describes a method of producing a Zn-Al-Mg coated steel sheet according to an embodiment of the present disclosure. An example of the method of producing a Zn-Al-Mg coated steel sheet includes: a process of preparing a base steel sheet; a process of immersing the base steel sheet in a coating bath having, in mass%, a chemical composition of Al: 0.5 % to 3.5 % and Mg: 0.5 % to 3.5 %, with the balance being Zn and inevitable impurities, to carry out a coating treatment on the base steel sheet and produce a coated steel sheet; a process of carrying out gas wiping on the coated steel sheet to adjust the coating weight; and then a process of cooling the coated steel sheet. Further, in the cooling process, the cooling is carried out at a cooling rate of 0.05 °C/s or more from after the gas wiping until a surface temperature of the coated steel sheet reaches 400 °C, and carried out in a vacuum atmosphere while the surface temperature of the coated steel sheet is from 300 °C to 100 °C. Further, the cooling of the coated steel sheet after the gas wiping until the surface temperature reaches 400 °C is preferably carried out in a N₂ atmosphere or a N₂ + 5 % H₂ atmosphere.

The type and thickness of the base steel sheet are as described above.

The coating bath used in production of the Zn-Al-Mg coated steel sheet has a chemical composition, in mass%, consisting of Al: 0.5 % to 3.5 % and Mg: 0.5 % to 3.5 %, with the balance being Zn and inevitable impurities. Further, the coating bath may contain, as optional additives, one or more selected from the group consisting of Si, Fe, Pb, Ti, Ni, Cu, Co, Mn, Cr, Mo, V, Sr, B, Bi, Cd, Sn, and REM (rare earth metals), in a total amount of 1.0 mass% or less. The explanation for each component in the coating bath is the same as the explanation of each component of the coated layer described above. The chemical composition of the coating bath is equivalent to the chemical composition of the coated layer.

When the temperature of the coating bath during the coating treatment is 410 °C or higher, the coating bath remains fully molten, effectively preventing bare spots. The temperature of the coating bath is therefore preferably 410 °C or higher. On the other hand, by keeping the coating bath temperature at 550 °C or lower, volatilization of coating bath components can be effectively prevented, enabling stable operation. The temperature of the coating bath is therefore preferably 550 °C or lower.

After the coating treatment, the coating weight is adjusted by gas wiping. There are no particular limitations on the conditions for the gas wiping, and standard methods can be used.

After the gas wiping, the coated steel sheet is cooled. In the cooling process from the gas wiping until the surface temperature of the coated steel sheet reaches 400 °C, the atmosphere in the process is oxygen-free, preferably a N₂ atmosphere or a N₂ + 5 % H₂ atmosphere. When oxygen is present in the atmosphere in this temperature range, oxidation of the coated surface progresses, making it easier for a thick oxide film to form on the surface, thus worsening the painting layer adhesion. Hereinafter, the temperature during cooling is based on the surface temperature of the coated steel sheet.

Further, in the cooling process from gas wiping until the surface temperature of the coated steel sheet reaches 400 °C, the cooling rate is preferably 0.05 °C/s or more. When the cooling rate is less than 0.05 °C/s, the line speed becomes extremely slow, resulting in a loss of productivity. On the other hand, there is no particular upper limit to the cooling rate in the temperature range. The cooling rate is preferably 100 °C/s or less.

For the same reasons, during the cooling process while the surface temperature of the coated steel sheet is from 400 °C to 300 °C, it is preferable to use a N₂ atmosphere or a N₂ + 5 % H₂ atmosphere.

During the cooling process while the surface temperature of the coated steel sheet is from 300 °C to 100 °C, the process is carried out under a vacuum atmosphere. Hereinafter, "vacuum atmosphere" means a vacuum level of 5 × 10⁻² to 2 × 10⁻¹ Pa in absolute pressure. The temperature range around 300 °C is the temperature range in which Zn-Al-Mg coating becomes a solid phase, and is also a temperature range where surface activity is high compared to room temperature. Therefore, an oxide film is likely to form on the surface in this temperature range, and since the formed oxide film remains on the surface even after cooling is complete, it is necessary to carry out cooling in a way that minimizes oxidation. During the cooling process, when the vacuum level in this temperature range exceeds 2 × 10⁻¹ Pa in absolute pressure, oxidation is promoted by the small amount of oxygen present, and a thick oxide film is formed on the coated surface. In addition, oxidation is more likely to occur in eutectic microstructures, which can easily lead to differences in oxide film thickness between surface microstructures. As a result, the painting layer adhesion deteriorates. Therefore, cooling in this temperature range is carried out in a vacuum atmosphere of 2 × 10⁻¹ Pa or less. On the other hand, in the cooling process, when the vacuum level in this temperature range is less than 5 × 10⁻² Pa in absolute pressure, expensive equipment such as a turbomolecular pump is required to achieve such a vacuum level, which is disadvantageous in terms of cost. Therefore, cooling in this temperature range is carried out in a vacuum atmosphere of 5 × 10⁻² Pa or more. Aside from radiative cooling, contact cooling, such as contact with a metal block having high thermal conductivity, may be used for cooling in a vacuum atmosphere.

For processes and conditions not described herein, conventional methods may be used.

### EXAMPLES

### [Test material preparation]

Using ultra-low-carbon mild steel (sheet thickness 0.8 mm) as the base steel sheets, coating treatment was carried out on the base steel sheets using coating baths having the same chemical compositions as the coated layer chemical compositions of the examples listed in Table 1. In each case, the coating bath temperature was 460 °C. After the coating treatment, gas wiping and cooling were carried out to produce coated steel sheets. During the cooling process from the gas wiping until the surface temperature of the coated steel sheet reached 400 °C, the cooling rate was 5 °C/s. Table 1 lists the atmosphere at each temperature range during cooling. For the examples in Table 1 where the atmosphere from 300 °C to 100 °C is defined as "vacuum", the vacuum level of the atmosphere was set to 8 × 10⁻² Pa in absolute pressure, and cooling was carried out by radiative cooling.

### [Table 1]

**Table 1**

| No. | Chemical composition of coated layer (mass%) | | | | Coated layer coating weight (g/m²) | Cooling atmosphere | | Coated layer surface | | | | Post-painting corrosion resistance | Painting layer adhesion | Classification |
|---|---|---|---|---|---|---|---|---|---|---|---|---|---|---|
| | Al | Mg | Other | Balance | | After gas wiping to 400 °C | 300 °C to 100 °C | Single-phase Zn microstructure | Eutectic microstructure | Average oxide film thickness (nm) | Standard deviation σ of oxygen intensity when average oxygen intensity is 1 | | | |
| 1 | 1.5 | 1.0 | - | Zn | 35 | N₂ | vacuum | ○ | Zn,Mg,Al | 35 | 0.17 | ⊚ | ⊚ | Example |
| 2 | 1.5 | 1.0 | - | Zn | 50 | N₂ | vacuum | ○ | Zn,Mg,Al | 42 | 0.17 | ⊚ | ⊚ | Example |
| 3 | 1.5 | 1.0 | - | Zn | 80 | N₂ | vacuum | ○ | Zn,Mg,Al | 47 | 0.25 | ⊚ | ○ | Example |
| 4 | 1.5 | 1.0 | - | Zn | 90 | N₂ | vacuum | ○ | Zn,Mg,Al | 51 | 0.31 | ⊚ | × | Comparative Example |
| 5 | 1.5 | 1.0 | - | Zn | 120 | N₂ | vacuum | ○ | Zn,Mg,Al | 59 | 0.34 | ⊚ | × | Comparative Example |
| 6 | 1.5 | 1.0 | - | Zn | 20 | N₂ | vacuum | ○ | Zn,Mg,Al | 33 | 0.13 | × | ⊚ | Comparative Example |
| 7 | 0.0 | 1.0 | - | Zn | 50 | N₂ | vacuum | ○ | Zn,Mg | 36 | 0.18 | × | × | Comparative Example |
| 8 | 1.0 | 1.0 | - | Zn | 50 | N₂ | vacuum | ○ | Zn,Mg,Al | 39 | 0.17 | ⊚ | ⊚ | Example |
| 9 | 2.0 | 1.0 | - | Zn | 50 | N₂ | vacuum | ○ | Zn,Mg,Al | 42 | 0.19 | ○ | ⊚ | Example |
| 10 | 3.0 | 1.0 | - | Zn | 50 | N₂ | vacuum | ○ | Zn,Mg,Al | 45 | 0.21 | ○ | ○ | Example |
| 11 | 5.0 | 1.0 | - | Zn | 50 | N₂ | vacuum | × | Zn,Mg,Al | 51 | 0.32 | × | × | Comparative Example |
| 12 | 1.5 | 0.0 | - | Zn | 50 | N₂ | vacuum | ○ | Zn,Al | 36 | 0.14 | × | ⊚ | Comparative Example |
| 13 | 1.5 | 2.0 | - | Zn | 50 | N₂ | vacuum | ○ | Zn,Mg,Al | 42 | 0.19 | ⊚ | ⊚ | Example |
| 14 | 1.5 | 3.0 | - | Zn | 50 | N₂ | vacuum | ○ | Zn,Mg,Al | 45 | 0.21 | ⊚ | ○ | Example |
| 15 | 1.5 | 5.0 | - | Zn | 50 | N₂ | vacuum | × | Zn,Mg,Al | 51 | 0.31 | × | × | Comparative Example |
| 16 | 0.0 | 0.0 | - | Zn | 50 | N₂ | vacuum | ○ | × | 36 | 0.16 | × | × | Comparative Example |
| 17 | 1.5 | 1.0 | - | Zn | 35 | N₂+5%H₂ | vacuum | ○ | Zn,Mg,Al | 38 | 0.17 | ⊚ | ⊚ | Example |
| 18 | 1.5 | 1.0 | - | Zn | 50 | N₂+5%H₂ | vacuum | ○ | Zn,Mg,Al | 42 | 0.17 | ⊚ | ⊚ | Example |
| 19 | 1.5 | 1.0 | - | Zn | 80 | N₂+5%H₂ | vacuum | ○ | Zn,Mg,Al | 49 | 0.25 | ⊚ | ○ | Example |
| 20 | 1.5 | 1.0 | - | Zn | 90 | N₂+5%H₂ | vacuum | ○ | Zn,Mg,Al | 52 | 0.31 | ⊚ | × | Comparative Example |
| 21 | 1.5 | 1.0 | - | Zn | 120 | N₂+5%H₂ | vacuum | ○ | Zn,Mg,Al | 60 | 0.34 | ⊚ | × | Comparative Example |
| 22 | 1.5 | 1.0 | - | Zn | 20 | N₂+5%H₂ | vacuum | ○ | Zn,Mg,Al | 34 | 0.13 | × | ⊚ | Comparative Example |
| 23 | 1.5 | 1.0 | - | Zn | 35 | air | vacuum | ○ | Zn,Mg,Al | 55 | 0.37 | × | × | Comparative Example |
| 24 | 1.5 | 1.0 | - | Zn | 50 | air | vacuum | ○ | Zn,Mg,Al | 59 | 0.37 | ○ | × | Comparative Example |
| 25 | 1.5 | 1.0 | - | Zn | 80 | air | vacuum | ○ | Zn,Mg,Al | 67 | 0.45 | ○ | × | Comparative Example |
| 26 | 1.5 | 1.0 | - | Zn | 90 | air | vacuum | ○ | Zn,Mg,Al | 69 | 0.51 | ○ | × | Comparative Example |
| 27 | 1.5 | 1.0 | - | Zn | 120 | air | vacuum | ○ | Zn,Mg,Al | 77 | 0.54 | ○ | × | Comparative Example |
| 28 | 1.5 | 1.0 | - | Zn | 20 | air | vacuum | ○ | Zn,Mg,Al | 51 | 0.33 | × | × | Comparative Example |
| 29 | 1.5 | 1.0 | - | Zn | 35 | N₂ | vacuum | ○ | Zn,Mg,Al | 38 | 0.23 | ○ | ○ | Example |
| 30 | 1.5 | 1.0 | - | Zn | 50 | N₂ | vacuum | ○ | Zn,Mg,Al | 42 | 0.23 | ○ | ○ | Example |
| 31 | 1.5 | 1.0 | - | Zn | 80 | N₂ | vacuum | ○ | Zn,Mg,Al | 49 | 0.29 | ⊚ | ○ | Example |
| 32 | 1.5 | 1.0 | - | Zn | 90 | N₂ | vacuum | ○ | Zn,Mg,Al | 52 | 0.37 | ○ | × | Comparative Example |
| 33 | 1.5 | 1.0 | - | Zn | 120 | N₂ | vacuum | ○ | Zn,Mg,Al | 60 | 0.40 | ⊚ | × | Comparative Example |
| 34 | 1.5 | 1.0 | - | Zn | 20 | N₂ | vacuum | ○ | Zn,Mg,Al | 34 | 0.19 | × | ⊚ | Comparative Example |
| 35 | 1.5 | 1.0 | - | Zn | 35 | N₂ | N₂ | ○ | Zn,Mg,Al | 42 | 0.31 | × | × | Comparative Example |
| 36 | 1.5 | 1.0 | - | Zn | 50 | N₂ | N₂ | ○ | Zn,Mg,Al | 48 | 0.36 | ○ | × | Comparative Example |
| 37 | 1.5 | 1.0 | - | Zn | 80 | N₂ | N₂ | ○ | Zn,Mg,Al | 59 | 0.44 | ○ | × | Comparative Example |
| 38 | 1.5 | 1.0 | - | Zn | 90 | N₂ | N₂ | ○ | Zn,Mg,Al | 63 | 0.50 | ○ | × | Comparative Example |
| 39 | 1.5 | 1.0 | - | Zn | 120 | N₂ | N₂ | ○ | Zn,Mg,Al | 75 | 0.53 | ○ | × | Comparative Example |
| 40 | 1.5 | 1.0 | - | Zn | 20 | N₂ | N₂ | ○ | Zn,Mg,Al | 36 | 0.32 | × | × | Comparative Example |
| 41 | 1.5 | 1.0 | - | Zn | 35 | N₂ | air | ○ | Zn,Mg,Al | 77 | 0.38 | × | × | Comparative Example |
| 42 | 1.5 | 1.0 | - | Zn | 50 | N₂ | air | ○ | Zn,Mg,Al | 92 | 0.37 | × | × | Comparative Example |
| 43 | 1.5 | 1.0 | - | Zn | 80 | N₂ | air | ○ | Zn,Mg,Al | 124 | 0.39 | ○ | × | Comparative Example |
| 44 | 1.5 | 1.0 | - | Zn | 90 | N₂ | air | ○ | Zn,Mg,Al | 134 | 0.41 | ○ | × | Comparative Example |
| 45 | 1.5 | 1.0 | - | Zn | 120 | N₂ | air | ○ | Zn,Mg,Al | 165 | 0.52 | ○ | × | Comparative Example |
| 46 | 1.5 | 1.0 | - | Zn | 20 | N₂ | air | ○ | Zn,Mg,Al | 61 | 0.34 | × | × | Comparative Example |
| 47 | 1.5 | 1.0 | - | Zn | 10 | N₂ | air | ○ | Zn,Mg,Al | 51 | 0.29 | × | × | Comparative Example |
| 48 | 1.5 | 1.0 | Si:0.5 | Zn | 35 | N₂ | vacuum | ○ | Zn,Mg,Al | 42 | 0.17 | ⊚ | ⊚ | Example |
| 49 | 1.5 | 1.0 | Fe:0.5 | Zn | 35 | N₂ | vacuum | ○ | Zn,Mg,Al | 42 | 0.17 | ⊚ | ⊚ | Example |
| 50 | 1.5 | 1.0 | Fe:1.0 | Zn | 35 | N₂ | vacuum | ○ | Zn,Mg,Al | 42 | 0.17 | ⊚ | ⊚ | Example |
| 51 | 1.5 | 1.0 | Si:0.5, Fe:0.5 | Zn | 35 | N₂ | vacuum | ○ | Zn,Mg,Al | 42 | 0.17 | ⊚ | ⊚ | Example |
| 52 | 1.5 | 1.0 | Ni:0.5 | Zn | 35 | N₂ | vacuum | ○ | Zn,Mg,Al | 42 | 0.17 | ⊚ | ⊚ | Example |
| 53 | 1.5 | 1.0 | Cr:0.5 | Zn | 35 | N₂ | vacuum | ○ | Zn,Mg, Al | 42 | 0.17 | ⊚ | ⊚ | Example |
| 54 | 1.5 | 1.0 | Sr:0.5 | Zn | 35 | N₂ | vacuum | ○ | Zn,Mg,Al | 42 | 0.17 | ⊚ | ⊚ | Example |
| 55 | 1.5 | 1.0 | Sn:0.5 | Zn | 35 | N₂ | vacuum | ○ | Zn,Mg,Al | 42 | 0.17 | ⊚ | ⊚ | Example |
| 56 | 1.5 | 1.0 | REM:0.5 | Zn | 35 | N₂ | vacuum | ○ | Zn,Mg,Al | 42 | 0.17 | ⊚ | ⊚ | Example |
| 57 | 1.5 | 1.0 | Pb:0.5 | Zn | 35 | N₂ | vacuum | ○ | Zn,Mg,Al | 42 | 0.17 | ⊚ | ⊚ | Example |
| 58 | 1.5 | 1.0 | Ti:0.5 | Zn | 35 | N₂ | vacuum | ○ | Zn,Mg,Al | 42 | 0.17 | ⊚ | ⊚ | Example |
| 58 | 1.5 | 1.0 | Cu:0.5 | Zn | 35 | N₂ | vacuum | ○ | Zn,Mg,Al | 42 | 0.17 | ⊚ | ⊚ | Example |
| 59 | 1.5 | 1.0 | Co:0.5 | Zn | 35 | N₂ | vacuum | ○ | Zn,Mg,Al | 42 | 0.17 | ⊚ | ⊚ | Example |
| 59 | 1.5 | 1.0 | Mn:0.5 | Zn | 35 | N₂ | vacuum | ○ | Zn,Mg,Al | 42 | 0.17 | ⊚ | ⊚ | Example |
| 60 | 1.5 | 1.0 | Mo:0.5 | Zn | 35 | N₂ | vacuum | ○ | Zn,Mg,Al | 42 | 0.17 | ⊚ | ⊚ | Example |
| 60 | 1.5 | 1.0 | V:0.5 | Zn | 35 | N₂ | vacuum | ○ | Zn,Mg,Al | 42 | 0.17 | ⊚ | ⊚ | Example |
| 61 | 1.5 | 1.0 | B:0.5 | Zn | 35 | N₂ | vacuum | ○ | Zn,Mg,Al | 42 | 0.17 | ⊚ | ⊚ | Example |
| 61 | 1.5 | 1.0 | Bi:0.5 | Zn | 35 | N₂ | vacuum | ○ | Zn,Mg,Al | 42 | 0.17 | ⊚ | ⊚ | Example |
| 62 | 1.5 | 1.0 | Cd:0.5 | Zn | 35 | N₂ | vacuum | ○ | Zn,Mg,Al | 42 | 0.17 | ⊚ | ⊚ | Example |
| 62 | 1.0 | 1.0 | - | Zn | 70 | N₂ | N₂ | ○ | Zn,Mg,Al | 55 | 0.56 | ○ | × | Comparative Example |
| 63 | 2.5 | 3.0 | - | Zn | 70 | N₂ | N₂ | ○ | Zn,Mg,Al | 22. | 0.58 | ○ | × | Comparative Example |

| | | | | | | | | | | | | | | |
|---|---|---|---|---|---|---|---|---|---|---|---|---|---|---|
| Underlined: indicates value outside scope of present disclosure. | | | | | | | | | | | | | | |

For each example of coated steel sheet obtained, the coating weight of the coated layer, the single-phase Zn microstructure, and the eutectic microstructure were confirmed using the methods described above. The average oxide film thickness and the standard deviation σ of the oxygen intensity were determined, with the average value of the oxygen intensity taken as 1. The results are listed in Table 1. In Table 1, under the column for single-phase Zn microstructure, examples where single-phase Zn microstructure was confirmed are marked with " ○", and examples where single-phase Zn microstructure was not confirmed are marked with "×". Further, in the eutectic microstructure column of Table 1, examples where eutectic microstructure was confirmed are marked with elements detected in the eutectic microstructure, and examples where eutectic microstructure was not confirmed are marked with ''×".

For each example of coated steel sheet (test material) obtained, the post-painting corrosion resistance and painting layer adhesion were evaluated as follows.

### [Post-painting corrosion resistance]

A 70 mm × 150 mm test piece was cut from the test material, and the test piece was subjected to Zr chemical conversion treatment and electrodeposition coating. The Zr chemical conversion treatment was carried out under standard conditions using PLM2100, produced by Nihon Parkerizing Co., Ltd. The electrodeposition coating was carried out using GT150V, produced by Kansai Paint Co., Ltd., to achieve a painted film thickness of 10 µm, and the curing conditions were 170 °C held for 20 min. Next, the test pieces were subjected to a corrosion test (SAE-J2334), and corrosion status after 180 cycles was evaluated.

After the corrosion test, the test pieces were cross-cut, and the maximum bulge width on one side from the cross-cut portion was measured. Each example was evaluated according to the following criteria, with "⊚" or "○" indicating a pass. The evaluation results are listed in Table 1.
⊚: maximum bulge width on one side < 4.0 mm
○: 4.0 mm ≤ maximum bulge width on one side < 5.0 mm
×: 5.0 ≤ maximum bulge width on one side

### [Painting layer adhesion]

As part of the evaluation of painting layer adhesion, an evaluation of water-resistant secondary adhesion was carried out. A 70 mm × 150 mm test piece was cut from the test material, and the test piece was subjected to Zr chemical conversion treatment and electrodeposition coating under the same conditions as for the evaluation of post-painting corrosion resistance. Next, each test piece was immersed in pure water at 60 °C for 20 days.

After the test, the test piece was cross-cut using an NT cutter S or A type (produced by NT Incorporated) to form 100 grid squares (10 × 10) with 2 mm spacing. Afterward, tape conforming to JIS Z 1522 (Cellotape CT-12S, produced by Nichiban Co., Ltd.) was applied to the cross-cut section and rubbed three times to adhere the tape. The tape was peeled off at a 90° angle to the attached surface of the test piece, at a speed of 0.5 m/s or more, and the number of grid squares where peeling occurred was measured. Each example was evaluated according to the following criteria, with "⊚" or "○" indicating a pass. The evaluation results are listed in Table 1.
⊚: number of peeled off grid squares: 0 to 5
○: number of peeled off grid squares: 6 to 15
×: number of peeled off grid squares: 16 to 100

The results in Table 1 indicate that the Examples according to the present disclosure have superior post-painting corrosion resistance and painting layer adhesion than the Comparative Examples.

### INDUSTRIAL APPLICABILITY

According to the present disclosure, it is possible to provide a Zn-Al-Mg coated steel sheet having excellent post-painting corrosion resistance and painting layer adhesion, which can be applied to various uses such as automotive steel sheets.

### REFERENCE SIGNS LIST

- 10: single-phase Zn microstructure
- 20: eutectic microstructure

## Claims

1. A Zn-Al-Mg coated steel sheet comprising a base steel sheet and a coated layer formed on at least one side of the base steel sheet,
wherein the coated layer has a chemical composition, in mass%, containing Al: 0.5 % to 3.5 % and Mg: 0.5 % to 3.5 %, with the balance being Zn and inevitable impurities,
wherein a surface of the coated layer has a microstructure comprising a single-phase Zn microstructure and a eutectic microstructure,
wherein the eutectic microstructure comprises a Zn-Mg intermetallic compound phase and a Zn phase, and optionally comprises either or both of an Al phase and an Al-Mg intermetallic compound phase,
wherein the coating weight of the coated layer is 35 g/m² to 80 g/m²,
wherein an average oxide film thickness at the surface of the coated layer is 50 nm or less,
and wherein, when an average value of oxygen intensity at the surface of the coated layer is taken as 1, a standard deviation σ of the oxygen intensity is 0.30 or less.

2. The Zn-Al-Mg coated steel sheet according to claim 1, wherein the chemical composition of the coated layer further contains one or more selected from the group consisting of Si, Fe, Pb, Ti, Ni, Cu, Co, Mn, Cr, Mo, V, Sr, B, Bi, Cd, Sn, and REM, in a total amount of 1.0 mass% or less.
